

# UNITED STATES PATENT OFFICE.

HERMAN C. PFEIL, OF CAMDEN, NEW JERSEY.

## COMPOSITION FOR SURFACING FABRICS.

SPECIFICATION forming part of Letters Patent No. 246,633, dated September 6, 1881.

Application filed April 14, 1881. (No specimens.)

*To all whom it may concern:*

Be it known that I, HERMAN C. PFEIL, a citizen of the United States, residing in the city and county of Camden, State of New Jersey, 5 have invented a new and useful Improvement in Surfacing Fabrics for Printing Purposes, which improvement is fully set forth in the following specification.

The invention consists of a coating for cloth 10 and other fabrics formed of a composition of matter which readily permits printing thereon and retains the same, is of a glossy nature, and is not liable to crack or peel, is water-proof, and possesses other advantages, as will be hereinafter set forth.

In carrying out my invention, I take one pound wax, one gallon varnish, five pounds white zinc, white lead, or Cremnitz white or other white mineral. The white mineral is 20 ground with the varnish. The wax is heated, and when to a boiling point it is mixed with the combined varnish and mineral white, the mass being continually stirred, so as to thoroughly unite the ingredients, after which it is 25 strained and applied hot or cold by means of brushes, rollers, &c., to muslin, linen, canvas, or other suitable cloth or fabric, it being seen that the resultant surface of the fabric is of a uniform, smooth, glossy, and flexible nature, 30 and readily permits printing thereon, the color

taking in a superior manner and remaining durable and bright, and does not crack and peel. It is, moreover, enabled to withstand exposure to the weather, and may be washed or cleansed with cold or warm water without 35 injury.

The surface is well adapted to receive impressions from the finest steel and copper plate, as well as from lithographic plates, wood-cuts, ordinary type, &c.

The kind of varnish which I use is white varnish, and may be made from Zanzibar gum, 40 turpentine, and bleached linseed-oil.

I am aware that compositions have been made for varnishing purposes, consisting principally of litharge, beeswax, and oily substances; also, compositions consisting of zinc white, wax, and varnish, together with a variety of additional ingredients. These compositions I do not claim.

What I do claim is—

A white composition for surfacing fabrics and other flexible material for printing purposes, consisting of wax, white varnish, and mineral white thoroughly incorporated, sub- 45 50 55 stantially as set forth.

HERMAN C. PFEIL.

Witnesses:

JOHN A. WIEDERSHEIM,  
W. F. KIRCHER.